

## UNITED STATES PATENT OFFICE

2,304,037

## PROPELLENT EXPLOSIVE CHARGE

Thomas Thomson, Kilmarnock, Scotland, and Edward Whitworth, New York, N. Y., assignors to Imperial Chemical Industries Limited, a corporation of Great Britain

No Drawing. Application April 19, 1941, Serial No. 389,462. In Great Britain March 11, 1938

13 Claims. (Cl. 52—7)

This invention relates to the manufacture of colloided nitrocellulose propellant explosive charges, and more particularly to the provision of gun charges containing a constituent adapted to reduce or eliminate muzzle flash which has also the property of reducing metallic fouling by action of the hot gases on the projectile in the firearm.

The inclusion of a small proportion of certain alkali metal salts in propellant powder charges made from colloided nitrocellulose with or without the inclusion of nitroglycerine or other gelatinisers, whether of deterrent or non-deterrent nature, is known to have a strong effect in reducing the muzzle flash; and, in conditions favourable to the action of the alkali metal salt, the flash may even be suppressed altogether. The alkali metal salts hitherto employed for this purpose, however, have not been possessed of the property of reducing to any appreciable extent the metallic fouling of the rifled arms in which the propellant charge containing them is fired. Flash reducing compounds moreover tend to cause a falling off in the smokelessness of the propellant charge.

It is known that metallic fouling in rifled arms is reduced by the inclusion in the propellant charge of tin, or lead, or certain alloys or compounds of these metals. One method of employing such a metal or alloy consists in encasing the charge or a portion thereof in the metal foil. It has also been proposed to incorporate tin or lead compounds as ingredients during the manufacture of the propellant powder. It has been stated that the muzzle flash produced by the combustion of the powder gases is very considerably reduced when tin, tin alloys, or tin compounds are present in the propellant charge.

It is an object of our invention to provide an anti-muzzle flash type of gun charge having a reduced tendency to cause smoke. It is also an object of our invention to provide an anti-fouling type of gun charge having improved flashless characteristics. It is a further object of our invention to produce an anti-fouling type of gun charge having a reduced tendency to cause smoke. It is a still further object of our invention to provide a gun charge having an improved combination of anti-fouling, anti-flash and smokeless characteristics. It is a still further object of our invention to provide a colloided nitrocellulose propellant powder containing within its composition a compound conferring anti-fouling and anti-flash characteristics chemically compatible with the common ingredients present in smokeless powders, and which powder has

5 satisfactory storage properties. A still further object is to provide colloided nitrocellulose powders adapted for automatic firing arms, which powders have improved firing characteristics, and with which no muzzle attachment for the suppression of flash is required.

We have found that these and other objects are attained by the inclusion in the colloided nitrocellulose charge of an antimony compound containing a combined alkali metal. The antimony compound is desirably one free from halogens. The alkali metal antimony tartrates and their double salts with other alkali metal salts are conveniently used, for instance potassium antimony tartrate, commonly known as tartar emetic, lithium or sodium antimony tartrate, or the double salts of potassium antimony tartrate with potassium bitartrate, lithium nitrate, sodium nitrate or sodium sulphate. We prefer, however, to employ tartar emetic. The colloided nitrocellulose propellant powder may be a single base powder or a double base powder, and may include gelatinisers of a deterrent or non-deterrent nature in its composition and may, if desired, be surface moderated. Any of the common detergents such as esters, nitrocompounds, substituted ureas or urethanes of low volatility may be employed, for instance, di-alkyl phthalates, alkyl glycollates, alkyl tartrates, alkyl lactates, acetates of polyhydric alcohols, dinitrotoluene, mononitrotoluene, diaryl dialkyl ureas, and aryl aralkyl urethanes and aryl alkyl urethanes, may conveniently be employed. In the case of double base powders, nitroglycerine or other liquid nitrates of polyhydric alcohols may be employed with or without detergents.

40 In putting the invention into effect we may introduce an antimony compound into the propellant composition in a uniform manner during the manufacture of the latter, but a uniform distribution is not always essential to the success of the invention. Thus in the case of charges for heavy artillery it is possible to employ as part of the charge an ordinary colloided nitrocellulose propellant powder and as another part of the charge a propellant powder containing a very considerable proportion of tartar emetic. In some cases the tartar emetic may be applied to the surface of the grains of the propellant powder thereby enabling stocks of already manufactured propellant powders to be treated so as to improve their characteristics. In the application of the invention to propellant charges for small arms ammunition for machine guns and the like, the most practicable methods of introducing the tartar emetic or other antimony compound used in-

volves its distribution in a more or less uniform manner throughout the powder. It may be conveniently introduced into the composition of the charge before the commencement of the gelatinisation of the nitrocellulose.

The proportion of tartar emetic employed may conveniently be from about 1% to about 5% reckoned on the weight of the total charge. Although increasing the proportion of this compound increases the anti-fouling and flash reducing properties, the compound is not devoid of all tendency to increase the smoke, and it is found that between these limits a particularly favourable combination of properties results.

The invention finds particular application in small arms ammunition for use in machine guns and automatic rifles, the use of tartar emetic containing propellant powders for such ammunition effectively reduces the muzzle flash and ensures effective removal of metallic fouling from the bore of the firearm, and renders unnecessary the use of muzzle attachments for masking muzzle flash. This is an advantage since these attachments frequently give trouble owing to the accumulation of the metallic fouling in them. The colloided nitrocellulose powders containing tartar emetic have storage properties as good as similar powders from which the tartar emetic has been omitted.

The invention is illustrated by the following examples in which the parts are parts by weight.

#### Example 1

This example relates to the manufacture of a single base rifle powder. An amount of alcohol-dehydrated nitrocellulose containing 99 parts dry weight of nitrocellulose of 13.2 per cent nitrogen content is mixed with 3 parts tartar emetic that has been finely ground and sifted through a wire sieve having 100 meshes to the inch, British standard specification. The mixture is then colloided by the introduction in known manner of ether containing in solution one part diphenylamine. The colloid is pressed through a die and cut. It is then treated for solvent recovery and steeped in hot water, and is finally surface moderated with 3 parts dimethyl diphenyl urea and coated with graphite.

In a test carried out with a 0.303 inch short magazine Lee-Enfield rifle in which the barrel had been considerably shortened, a rifle powder so prepared gave no flash whatever when fired; whereas a powder made in similar fashion but from which the tartar emetic had been omitted, gave a brilliant flash. An analysis of the metallic deposits from 47 rounds of cupro-nickel jacketed bullets in 0.303 inch short magazine Lee-Enfield barrels fired with the rifle powder containing the tartar emetic and the same number of rounds fired with the powder from which it had been omitted gave as the total weight of metal fouling 0.05 gm. and 0.25 gm. respectively. The diminution in the effective bore diameter caused by the metal fouling at a point 20 inches up the barrel in the case of the powder containing the tartar emetic was only about one tenth of that observed in the case of the powder containing no tartar emetic.

#### Example 2

This example relates to the manufacture of a single base machine gun powder. An amount of alcohol dehydrated nitrocellulose containing 99 parts dry weight of nitrocellulose of 13.2 per cent nitrogen content is mixed with tartar emetic that has been finely ground and sifted through a wire

sieve having 100 meshes to the inch, British standard specification. The mixture is then colloided by the introduction of ether containing in solution one part of diphenylamine. The colloid is pressed through a die and cut. It is then treated for solvent recovery and steeped in hot water, and is finally surface moderated with a mixture of 3.5 parts dimethyl diphenyl urea and 3.5 parts dibutylphthalate and coated with graphite.

#### Example 3

This example relates to the manufacture of a double base machine gun powder. 29 parts nitroglycerine are mixed with 65 parts dry nitrocellulose of 13.1 per cent. nitrogen content. The resulting paste is colloided with a solution of 6 parts diethyl diphenyl urea in aqueous acetone and 3 parts of tartar emetic are added during the incorporation of these ingredients, which is carried out in a mixing machine at about 30° C. The resulting plastic is pressed through a die into cords which are subsequently stoved and reeled into a rope, which is finally cut to the desired grain length.

The advantages of the invention may be readily appreciated by the following table showing the results of a test carried out in a 1/2 inch Vickers machine gun using a 664 grain bullet having a solid gilding metal envelope, the number of rounds fired being 20, in which the results obtained on firing the powder of Example 2 are compared with those obtained on firing otherwise similar powders from the composition of which the tartar emetic has been omitted or replaced by certain hitherto known anti-fouling and anti-flash ingredients.

The first column of the table indicates the amount of anti-flash or anti-fouling ingredient used in making the colloided nitrocellulose powder for every 99 parts of the nitrocellulose. The second column indicates the amount of copper found by analysis in the barrel residues of the firearm, and the third column describes the appearance of the flash obtained. The fourth column indicates the order in which the various powders used approach freedom from smoke.

| Ingredient                                 | Copper | Flash           | Freedom  |
|--------------------------------------------|--------|-----------------|----------|
|                                            |        |                 | from     |
|                                            | Grams  |                 | smoke    |
| Nil                                        | 0.4080 | Large brilliant | 1) About |
| 1/2 parts tin                              | 0.2948 | do              | 1) equal |
| 3 parts tartar emetic                      | 0.1292 | None            | 3.       |
| 2 parts potassium bitartrate               | 0.2754 | do              | 4.       |
| 1/4 parts tin+2 parts potassium bitartrate | 0.1930 | do              | 5.       |

When antimony compounds containing a combined alkali metal other than tartar emetic are used, an amount having an antimony content equivalent to that of one to five parts tartar emetic may be conveniently employed for every 100 parts of the propellant explosive.

As many apparently widely different embodiments of the invention can be made without departing from the spirit and scope thereof, it must be understood that the invention is not limited to any specific embodiment except as defined in the appended claims.

We claim:

1. A colloided nitrocellulose propellant powder gun charge comprising an antimony compound free from halogens and containing a combined alkali metal.

2. A colloided nitrocellulose propellant powder gun charge comprising an alkali metal antimonyl tartrate.
3. A colloided nitrocellulose propellant powder gun charge comprising tartar emetic.
4. A small arms propellant powder comprising colloided nitrocellulose propellant powder having tartar emetic distributed homogeneously through it.
5. A small arms propellant powder comprising a single base colloided nitrocellulose powder having tartar emetic distributed homogeneously through it.
6. A colloided nitrocellulose propellant powder comprising tartar emetic and a deterrent.
7. A colloided nitrocellulose propellant powder, as claimed in claim 6 in which the powder is surface moderated with the deterrent.
8. A colloided nitrocellulose propellant powder gun charge comprising a double salt of an alkali metal antimonyl tartrate and another alkali metal salt free from halogens.
9. A colloided nitrocellulose propellant gun charge containing from about 1 to about 5 per cent. tartar emetic.
10. A colloided nitrocellulose propellant powder gun charge having an alkali metal antimonyl tartrate distributed unequally through it.
11. A colloided nitrocellulose propellant powder comprising a deterrent and from about 1 to about 5 per cent. tartar emetic.
12. A smokeless colloided nitrocellulose propellant powder to the surface of which tartar emetic has been applied.
13. A colloided nitrocellulose powder gun charge comprising an amount of an alkali metal antimonyl tartrate equivalent in its antimonyl content to about 1 to about 5 per cent. tartar emetic.

THOMAS THOMSON.  
EDWARD WHITWORTH.